

## UNITED STATES PATENT OFFICE

2,646,353

REMOVAL OF VOLATILE PRODUCTS FROM  
PHOTOGRAPHIC EMULSIONS

George D. Hill and Rudolph E. Damschroder,  
Rochester, N. Y., assignors to Eastman Kodak  
Company, Rochester, N. Y., a corporation of  
New Jersey

No Drawing. Application December 31, 1948,  
Serial No. 68,744

3 Claims. (Cl. 95—7)

## 1

This invention relates to methods of preparing photographic silver halide emulsions and more particularly to a process of forming photographic emulsions wherein by-products are removed, for example, by means of vacuum.

It is well known in the art of photographic emulsion making that it is desirable to remove soluble salts resulting from the emulsion-making reactions, especially in those cases where the emulsion is designed for coating on transparent supports. Equally well known are emulsions of the type where ammonia is used in making the emulsion and is present in the reaction mixture after formation of the silver halide. In such processes the ammonia and any soluble salt present are customarily removed by shredding the emulsion and washing out the ammonia with water.

In such processes it is customary in the art, after precipitation of silver halide in the presence of a protective colloid, to chill the emulsion so that it can be cut up and shredded, following which the pieces are washed for the desired time to remove salts or dissolved material such as ammonia. Frequently this process requires many hours to effect the removal of salt, and is performed in batches in crocks, tanks, shredding machines and other equipment for chilling, shredding and washing the emulsion.

It is, therefore, one object of our invention to provide a new method of making a photographic emulsion. Another object is to provide novel methods of making and purifying a photographic emulsion. A still further object is to provide an economical continuous process of forming a photographic emulsion of optimum quality. Further objects of our invention will become apparent from consideration of the following description.

Our invention resides in, and the objects of our invention are accomplished by, reacting an aqueous ammonia solution of a silver salt, such as silver nitrate, with a water-soluble halide and removing the nitrogenous product, such as ammonia, from the reaction mixture by means of vaporization, such as by vacuum.

It will be apparent that when we use vacuum for removal of a volatile material dissolved in a reaction mixture, a very economical process is made available. We have found that when vacuum is employed to remove ammonia or other volatile compounds from the emulsions of our invention, a decided saving in time, materials and manpower is effected. Also the photographic quality obtainable from the emulsion so treated

is comparable to that obtainable by the washing technique of the prior art. The quality of the product can be higher, especially since there is no possibility of emulsion contamination by impurities of the wash water usually used and because better control means are made available. A further advantage is the fact that the process may be continuous in operation. The above advantages will become more apparent by consideration of the following detailed description of our invention.

The emulsions which are adaptable to use in our invention are formed by reacting a silver salt such as silver nitrate dissolved in an excess of ammonia or lower aliphatic amine solution, with a water-soluble halide salt such as an alkali metal halide, ammonium halide, or alkyl-substituted ammonium halide of the following structure:



where X is a halogen atom and R, R<sub>1</sub>, R<sub>2</sub> and R<sub>3</sub> each represents a hydrogen atom or an alkyl group having from one to four carbon atoms, and in which the sum of the carbon atoms is not over four. Thus, water-soluble halides which we can use are the common ammonium halides, for example, ammonium chloride, bromide, or iodide and methyl ammonium bromide or chloride, dimethyl or trimethyl ammonium halides, ethyl ammonium bromide or chloride and quaternary ammonium halides. We can use one or more of such halides or other water-soluble metal halides, together and particularly in conjunction with an iodide such as sodium or ammonium iodide. Generally the total number of carbon atoms in the alkyl group or alkyl groups attached to the nitrogen atom in the above formula is less than five because the amines of more carbon atoms resulting from the emulsion reaction are not sufficiently volatile to be removed by vacuum. Accordingly, we prefer to use hydrogen halides, alkali metal, ammonium or methyl ammonium halides in our invention.

The following examples are given as illustrative of our invention:

## Example 1

One kg. of silver nitrate dissolved in a 10% excess of ammonia and made up with water to a total volume of 10 liters was added to a solution containing 1 kg. of gelatin and 700 grams of potassium bromide in 10.5 liters of solution. The resulting mixture was passed through a vac-

uum system to remove the excess ammonia until there remained not more than 22 gms. of ammonia per kg. of silver nitrate used. From this point on, the emulsion was treated according to conventional procedures known in the art, exclusive of washing, for preparing a finished emulsion suitable for coating on a paper support. This can be accomplished by adding 350 g. additional gelatin and adjusting the pH to 9.15 before coating on a paper support. After evacuation, additions may be made of gelatin or other protein vehicles or vehicles such as hydrolyzed cellulose esters of polyvinyl alcohol and ripening or digesting operations customary in the art may now be carried out.

*Example 2*

The following solutions were prepared in the usual manner:

I

|                         |       |      |
|-------------------------|-------|------|
| Gelatin (16.8% aqueous) | grams | 6080 |
| Potassium bromide       | do    | 665  |
| Potassium iodide        | do    | 10.3 |
| Water                   | cc    | 9530 |

II

|                               |       |      |
|-------------------------------|-------|------|
| Silver nitrate                | grams | 1000 |
| Monomethylamine (25% aqueous) | cc    | 3320 |
| Water                         | cc    | 9000 |

Solutions I and II were mixed as rapidly as possible at a temperature of 120° F. After a short interval at 117° F., the emulsion was passed through an outgassing apparatus and monomethylamine was partially removed until the pH was 10.35. The resulting emulsion was treated, ripened or digested and coated on a paper support at pH 9.15 in the manner well known in the photographic emulsion-making art exclusive of washing.

In preparing the emulsions such as above described, it is not necessary to use gelatin as the peptizing material, but other peptizing hydrophilic colloids may be used such as polyacrylamide or imide resins as disclosed in the Lowe et al. U. S. patent application Serial No. 685,375, filed July 22, 1946 now U. S. Patent No. 2,541,474 granted February 13, 1951, particularly the polyacrylamides containing 15 to 20 per cent combined acrylimide and imidized polyacrylamides containing 30 to 60 per cent combined acrylimide and 4 to 12 per cent combined acrylic acid described therein; modified proteins e. g. derivatives of casein, soybean protein, blood albumin, egg albumin, etc., obtained by reaction of these proteins with sulfonyl chlorides, carboxylic acid chlorides, anhydrides, etc., prior or subsequent to oxidative hydrolysis with, for example, peroxide as disclosed in Lowe et al. U. S. patent application Serial No. 768,480, filed August 13, 1947, and similar materials.

In a manner similar to that described in the above examples, we can use a solution of another silver salt such as silver carbonate, citrate, tartrate, acetate, sulfate, etc., and cause it to react with an alkali metal or ammonium halide and the nitrogenous by-products resulting are removed as by evacuation of the reaction mixture, washing not being employed. Therefore, according to our invention, when an aqueous ammonia solution of a silver salt is reacted with one of the halides, the resulting reaction mixture contains silver halide, volatile nitrogenous products as ammonia or an amine, and a water-soluble, non-

volatile salt such as an alkali metal salt containing the anion of the silver salt used.

According to the spirit of our invention, as illustrated above, when the silver salt is dissolved with a solution containing ammonia or an amine, an "ammoniacal" solution is formed by which term we mean to include solutions containing silver salt and either ammonia or an amine such as methyl, ethyl, propyl, dimethyl, and diethyl amines, any of which can be used for dissolving the silver salt prior to reaction with the halide salt.

In order to remove ammonia from the emulsion systems described, we have found it advisable to supply heat to the liquid being evacuated to compensate for the drop in temperature arising from the heat supplied for vaporization and the tendency for the rate of removal of ammonia to fall with drop in temperature thereby. The rate and extent of the removal of moist ammonia is, of course, controlled on the one hand by the peculiarities of the vacuum equipment and the flow of the liquid through it, which naturally depends somewhat on the capacity of the vacuum-pumping means. We have found that the most useful range of operation includes a range of pressure in the vacuum system of from 20 to 30 mm. of mercury, and when heat is supplied to the liquid film by means of a water jacket, a range of temperature from 60 to 80° C. in the jacket is most satisfactory. However, in a typical all-glass installation using water jackets and aspirator pumps, appreciable amounts of ammonia are quickly removed with the water temperature at 40° C. and a vacuum pressure of 90 mm. As is apparent, the most suitable or desirable conditions of rate of flow, temperature and pressure for a given apparatus are readily determinable but depend on definite characteristics of that equipment. After we determine the characteristics of the vacuum system, that is, its rate of removal of ammonia, or volatile dissolved product, we are next governed by matters of economy and photographic quality. That is, in certain instances where it is desired to remove substantially all of the ammonia from the reaction mixture, we can do so by selection of the optimum conditions of temperature, pressure and rate of flow through the evacuation chamber. In other cases where we have use for an emulsion from which all of the ammonia has not been removed, we naturally increase the rate of flow or lower temperature or increase the pressure, or we can vary one or more of these conditions at the same time, as will be apparent to those skilled in the art.

Since the grain characteristics and photographic properties of an ammoniacal emulsion are controlled by the concentration, temperature and time of the ammonia solutions in contact with the silver salt, it is desirable to operate our invention in such a way that the grains of silver salt are ripened and the ammonia is reduced in concentration to less than 22 grams per kilogram of silver nitrate converted to silver halide in a total time of less than 2 hours. This we may accomplish either by short ripening and slow removal or by more prolonged ripening and fast removal or short ripening and fast removal.

One advantage and unique feature of our process is now apparent. Having determined the operating characteristics of the emulsion-making system, we may remove practically any quantity of ammonia or volatile material from the silver halide reaction mixture. If we desire an emul-

sion having all of the characteristics derivable from a similar well-washed emulsion, we remove that amount of ammonia which corresponds to washing, and it is not necessary to remove dissolved salts to obtain this quality. Similarly, if desired, we remove less ammonia with the result, among other things, of obtaining an appreciable increase in the output of the evacuation system. Since sensitometric characteristics and photographic quality are of prime importance, we remove an amount of ammonia commensurate with utmost economy and proven dictates of photographic quality.

It is to be noted that our process is unique in that it removes ammonia in the presence of a soluble salt such as ammonium or alkali metal nitrate also contained in the reaction mixture. When the resultant composition is ripened, digested or treated in the same manner as would be normal had washing been employed, the finished emulsion has just as good photographic characteristics in spite of the fact that dissolved salts were not removed, particularly when such emulsions are coated on supports such as paper. Thus there is made available a process whereby we can remove practically all or part of the ammonia associated with the silver halide then, if desired, we can add ammonia in definite quantities during finishing operations, but we are not limited, as by washing methods, to the grain characteristics obtained while the silver halide is in contact with ammonia during a washing period.

Finished emulsions having desirable photographic qualities can be made by removing ammonia until a range of from about 0 to 22 grams of ammonia per kilogram of silver nitrate used in making the emulsion and converted to silver halide, remains associated with the silver halide. That is, the volatile nitrogen compounds present in the reaction mixture are removed until the molecular equivalent amount of the nitrogen compound remaining in the emulsion is equal to less than about 22 grams of ammonia per kilogram of silver nitrate used.

It will be apparent that when an alkyl-substituted ammonium halide is used, the efficiency of our process may be lowered principally because of the higher boiling point of the aliphatic amine formed in the reaction and which is to be removed from the reaction mixture. In such cases we may desire to wash the material from the emulsion with or without previous evacuation treatment as we can do when water-soluble halides or ammonium or alkali metal halides are used. Similarly, when the nitrogenous product such as ammonia is highly volatile, we may partially or completely dispense with vacuum treatment and remove the ammonia by passing a strong current of air over the surface of the reaction mixture, by means of efficient liquid film vapor exchangers.

In certain cases it may be desirable to carry out the evacuation of the emulsion before or after ripening or digesting or other steps known to emulsion making. However, we prefer to remove a material such as ammonia prior to ripening of the emulsion. Our process is especially adaptable to removing the ammonia just after or as soon after formation of silver halide as it possible and, therefore, may readily be adapted to a continuous manufacturing process. We merely precipitate the halide as described, then conduct the silver halide reaction mixture in a continuous manner from the reaction chamber to the evacu-

ation chamber, and if the evacuation system is operated at a fairly low capacity, we use a temporary holding tank therebetween. An advantage of so operating lies in the fact that the emulsion has no appreciable opportunity to ripen in the presence of an undesirable quantity of ammonia, and it is removed much more quickly than could be done by washing. Therefore, silver halide grain size is capable of being controlled more readily than previously by operating according to our invention.

It is to be understood that the disclosure herein is by way of example, and that we consider as included in our invention all modifications and equivalents falling within the scope of the appended claims.

What we claim is:

1. The method of making a photographic silver halide emulsion which comprises reacting in an excess of aqueous ammoniacal solution in the presence of a peptizing hydrophilic colloid for silver halide, substantially equivalent quantities of silver nitrate and a water-soluble halide salt selected from the group consisting of alkali metal halides, ammonium halides and methylamine halides, to yield silver halide, a volatile nitrogenous product and a water-soluble non-volatile salt product, removing said volatile nitrogenous product from said emulsion only by passing the emulsion as a thin film of liquid through a chamber maintained at a pressure of from about 20-90 mm. of mercury and a temperature of from about 40-80° C. until the molecular equivalent amount of the nitrogenous product remaining in the emulsion is equal to less than about 22 grams of ammonia per kilogram of silver nitrate originally used in making the emulsion and converted to silver halide, and digesting the emulsion, the removal of nitrogenous product and digestion being effected within less than two hours.
2. The method of making a photographic silver halide emulsion which comprises reacting in an excess of aqueous ammoniacal solution in the presence of a peptizing hydrophilic colloid for silver halide, substantially equivalent quantities of silver nitrate with an alkali metal halide, to yield silver halide, a volatile nitrogenous product and alkali metal nitrate product, removing said volatile nitrogenous product from said emulsion only by passing the emulsion as a thin film of liquid through a chamber maintained at a pressure of from about 30-90 mm. of mercury and a temperature of from about 40-80° C. until the molecular equivalent amount of the nitrogenous product remaining in the emulsion is equal to less than about 22 grams of ammonia per kilogram of silver nitrates originally used in making the emulsion and converted to silver halide, and digesting the emulsion, the removal of nitrogenous product and digestion being effected within less than two hours.
3. The method of making a photographic silver halide emulsion which comprises reacting in an excess of aqueous ammonia solution in the presence of a peptizing hydrophilic colloid for silver halide, substantially equivalent quantities of silver nitrate with an ammonium halide, to yield silver halide, ammonia and ammonium nitrate, removing ammonia from said emulsion only by passing the emulsion as a thin film of liquid through a chamber maintained at a pressure of from about 20-90 mm. of mercury and a temperature of from about 40-80° C. until the amount of ammonia remaining in the emulsion is equal to less than about 22 grams of ammonia.

per kilogram of silver nitrate originally used in making the emulsion and converted to silver halide, and digesting the emulsion, the removal of ammonia and digestion being effected within less than two years.

GEORGE D. HILL.  
RUDOLPH E. DAMSCHRODER.

## References Cited in the file of this patent

## UNITED STATES PATENTS

| Number    | Name           | Date           |
|-----------|----------------|----------------|
| 1,861,918 | Hickman        | July 7, 1932   |
| 2,158,219 | Claus          | May 16, 1939   |
| 2,256,356 | Russell et al. | Sept. 16, 1941 |

5

10

8  
FOREIGN PATENTS

| Number  | Country       | Date          |
|---------|---------------|---------------|
| 3,782   | Great Britain | 1873          |
| 477,315 | Great Britain | Mar. 23, 1936 |

## OTHER REFERENCES

Wall: "Photographic Emulsions," published by American Photographic Publishing Co., 1929, pp. 221, 222, 223, 225 and 226, cited.

The Amateur Photographer, volume 18, pp. 223, 224, 242 and 243.

The British Journal of Photography (1883), pages 41, 42 and 71.